

## UNITED STATES PATENT OFFICE.

CHARLES ELLISON MACQUIGG, OF FLUSHING, NEW YORK, ASSIGNOR TO ELECTRO METALLURGICAL COMPANY, OF NIAGARA FALLS, NEW YORK, A CORPORATION OF WEST VIRGINIA.

## CARBONIZING BOX OR THE LIKE.

No Drawing. Application filed November 21, 1921. Serial No. 516,867.

To all whom it may concern:

Be it known that I, CHARLES ELLISON MACQUIGG, a citizen of the United States, residing at Flushing, Long Island, in the county of Queens and State of New York, have invented certain new and useful Improvements in Carbonizing Boxes or the like, of which the following is a specification.

10 This invention relates to alloys for use in the manufacture of articles required to resist corrosion and disintegration at high temperatures. More particularly the invention consists of the addition of copper to alloys of chromium with metals of the iron group for use in the connection mentioned.

15 Alloys of chromium with one or more of the metals of the iron group, especially iron, nickel and cobalt, are much used because of

20 their resistance to oxidation, corrosion and structural distortion at high temperatures. For some industrial purposes, not only are these qualities required, but the alloy must be capable also of withstanding carbonizing

25 influences without deterioration. After articles made from alloys of the kind specified have been used for a time in operations where a material portion of their surface is subjected to carbon or carbonizing gases at

30 elevated temperatures, cracking or spalling frequently occurs when the articles undergo the rapid temperature changes incident to commercial heat treatments. In this way they are often rendered useless long before corrosion, scaling, and the like have substantially impaired the alloy.

Such disintegrative effects are encountered particularly in carbonizing or cementation boxes, and it is the principal object of

40 my invention to provide improved boxes of this type. It will be understood, however, that the invention is applicable in general to the manufacture of articles to be subjected to carbonizing conditions.

45 My investigations tend to show that the cracking and spalling of articles formed from chromium-iron alloys and the like, under the conditions referred to, may be due to absorption of carbon by portions of the alloy article, or to the formation of metal car-

50 bids in localized areas. I attribute the break-

age of the article when it undergoes changes in temperature, to the internal stresses set up by differences in the coefficients of expansion of the carbonized and uncarbonized portions.

According to my invention, disintegration of articles formed from such alloys is minimized or eliminated by the addition of a metal having the property of preventing the destructive effects of carbonizing conditions, probably through inhibiting carbonization, without substantially impairing the strength or corrosion-resisting properties of the alloy. Copper is the preferred metal for effecting these results. The addition of copper seems to produce a favorable effect on the resistance of the alloys to oxidation and corrosion, and does not interfere with their machining or forging.

Even relatively small quantities of copper have a desirable protective action on chromium alloys subjected to carbonizing conditions, but in general the best results are obtained by adding copper in the maximum amount which will alloy with the other metals. This amount is a function of the composition of the alloy. It may be said, however, that for alloys containing 20% or more of chromium, the limit of solubility of copper is of the order of magnitude of 5 to 7%. Copper may be added with advantage to any of the oxidation-resistant alloys of chromium with metals of the iron group when such alloys are to be used for the manufacture of carbonizing boxes or other devices intended for use under conditions favoring carbon absorption.

I claim:

1. An article of manufacture composed of an alloy comprising chromium and a metal of the iron group, in amounts adapted to form an oxidation-resisting composition, and sufficient copper to render the composition resistant to carbonization.

2. An article of manufacture adapted to resist carbonization and composed of an alloy comprising chromium and iron in amounts adapted to form an oxidation-resistant body and copper in amount approximating its maximum solubility in the alloy.

3. An article of manufacture adapted to

resist carbonization and composed of a ferrous alloy containing chromium in amount not less than 20%, and 5 to 7% copper.

4. A carbonizing box or the like composed of an oxidation-resisting chromium alloy containing copper in amount sufficient to render the box resistant to carbonization.

5. A carbonizing box or the like, com-

posed of an alloy comprising chromium and iron in amounts adapted to form an oxidation-resisting body and copper in amount approximating its maximum solubility in the alloy.

In testimony whereof, I affix my signature.

CHARLES E. MACQUIGG.